# EUROPEAN PATENT SPECIFICATION

(11) **EP 2 428 126 B1**
(45) Date of publication and mention of the grant of the patent: **21.11.2018**
(21) Application number: 11180945.5
(22) Date of filing: 12.09.2011
(51) Int. Cl.: A24B 13/00

(54) **Smokeless oral product**
Rauchfreies orales Produkt
Produit oral sans fumée

(30) Priority: 13.09.2010 GB 201015216
(43) Date of publication of application: 14.03.2012
(73) Proprietor: British American Tobacco (Investments) Limited, London WC2R 3LA (GB)
(72) Inventor: Mola, Michele, London, WC2R 3LA (GB)
(74) Representative: D Young & Co LLP

(56) References cited:
- EP-A1- 2 529 634
- WO-A1-2011/093304
- US-A1- 2004 118 421
- US-A1- 2010 218 779

## Description

### Field of the Invention

The present invention relates to a smokeless product for oral administration.

### Description

Smokeless oral products are known. They comprise smokeless materials, such as smokeless tobacco, that are designed to be placed in the oral cavity of a user for a limited period of time. In use, substances from the smokeless material are adsorbed into the user's bloodstream via the mucosal membranes. Swedish-style snus is a popular smokeless oral product comprising tobacco.

Document US2010/0218779 A1 discloses an oral tobacco pouch providing controlled flavour release and including a web containing a filling material, the filling material including tobacco material.

Document US2004/0118421 A1 discloses a tobacco product for use in the mouth, said product comprising a multi-layer structure wherein the product comprises at least one load layer and a construction layer.

A common method of providing a smokeless oral product is to seal a moist, finely ground material in a permeable pouch. The pouch holds the material in place, while at the same time allowing substances such as flavours and nicotine to diffuse through the pouch and into the mouth of the user for absorption through the user's mucous membranes.

Conventional pouches for use with smokeless oral products are generally formed from viscose which is a regenerated cellulose material. The raw material used in the production of viscose is purified cellulose, which is generally obtained from specially processed wood pulp. However, although trees are a renewable source of raw material, they are not rapidly replaced, and therefore it would be advantageous to provide a material that is produced from a renewable source that is readily regenerated, such as an annual crop. In addition, the production of viscose can generate pollution due to the effects of carbon disulfide and other by-products of the process.

Furthermore, conventional pouch materials such as viscose may become stained and discoloured due to the moisture present in smokeless materials. Such unsightly markings can make the product unappealing to the user.

In addition, conventional pouch materials are generally composed of fibre web materials. Such materials have the disadvantage of having mechanical properties that are directionally specific, in other words, the material is strong when stressed in one direction but weaker when stressed in another. It would be advantageous to provide a material having equivalent mechanical properties in all directions to provide greater control and flexibility in the manufacturing process.

The present invention seeks to provide a smokeless oral product that overcomes or substantially alleviates the problems described above.

### Statements of the Invention

According to a first aspect of the present invention, a smokeless oral product according to claim 1 is provided. The smokeless oral product comprises a permeable pouch comprising a woven material, and the pouch contains smokeless material.

The smokeless material may comprise a smokeless tobacco material, which may be Swedish-style snus.

The permeable pouch may comprise both woven and non-woven material, or may comprise a composite material comprising both woven and non-woven material. The material comprises polylactide or polyolefin material.

According to a second aspect of the present invention, a method of producing a smokeless oral product according to claim 6 is provided. The method comprises providing a permeable pouch comprising a woven material and the pouch contains smokeless material, such as smokeless tobacco material.

The method may comprise sealing the material using heat-melt or ultrasonic weld techniques.

### Drawings

Embodiments of the invention are described, by way of example only, with reference to the accompanying drawings in which:
Figure 1 is a diagram illustrating a method of producing a smokeless oral product comprising the use of a heat-weld technique;
Figure 2 depicts a smokeless oral product comprising a woven material which is ultrasonically sealed.

### Detailed Description of the Invention

The present invention is directed towards a smokeless oral product comprising a permeable pouch. The pouch is intended to contain smokeless material, such as smokeless tobacco or tobacco substitute material. The smokeless oral product is used by being placed in the mouth of the user, for example in the side of the mouth between the cheek and gums. In use, flavours and other substances from the smokeless material diffuse out of the pouch and into the mouth of the user.

Consequently, the form and dimensions of the pouch are limited only by the capacity to fulfil this function.

The pouch should generally be of a size that is small enough to be comfortably accommodated in the mouth of the user; however, it should also be large enough to retain a suitable quantity of smokeless material.

Equally, the shape of the pouch is limited only by functional considerations. The pouch should be of a shape that is comfortable for the user.

According to some embodiments, the pouch comprises only front and back surfaces. The two surfaces may comprise separate pieces of material, or alternatively, the two surfaces may be formed from a single sheet of material. In some embodiments, a single section of material that is folded to form the front and back surfaces is used to form the pouch as this reduces the number of seams required. In some embodiments, the material is produced in a single tubular form, and this obviously further reduces the number of seams required and is therefore preferred.

The front and back surfaces may be the same or different sizes and shapes. The two annealed surfaces may be any shape, including regular shapes such as square, oval, triangular etc, or irregular shapes, having straight or curved edges. In preferred embodiments, however, the surfaces are the same shape and size and are rectangular, or circular.

In alternative embodiments, the pouch may be in the form of a polyhedron, for example, a tetrahedron or hexahedron (box-form), or a cylinder.

One or all of the surfaces of the pouch may be porous and may comprise woven material. In addition, a single surface may comprise regions of porous and non-porous material, any of which may comprise woven material.

In embodiments in which the pouch is generally rectangular in shape, the pouch may be between 20mm and 50mm in length. For example, the pouch may be between 25mm and 30mm, between 30mm and 35mm, or between 35mm and 45mm in length. Preferred lengths for the pouch are 28mm, 33mm, and 42mm. The pouch may be between 10mm and 20mm in width, and is preferably between 11mm and 14mm, or between 16mm and 19mm in width. Preferred widths for the pouch are 12mm and 18mm.

The pouch may be configured to have a flexible shape that is capable of being manipulated by the user to provide an optimal arrangement for comfortable use.

The pouch may be configured so that it is capable of providing for the passage of saliva and other substances, such as tobacco constituents, into and out of the pouch. For example, in some embodiments, the pouch is composed entirely of a permeable material which may comprise a woven material. In this case, diffusion may occur across substantially the entire surface of the pouch.

In other embodiments, a proportion of the material comprising the pouch is impermeable to the passage of saliva or other substances, and according to these embodiments, the pouch may be provided with at least one porous surface, which may comprise a woven material. For example, in the case of a polyhedral or cylindrical pouch, one or more of the surfaces of the pouch may be formed from a permeable material which may comprise polylactide (PLA) or polyolefin (PO) material.

In alternative embodiments, one or more non-porous surfaces or regions of the pouch may comprise PLA material.

### Manufacture of the pouch

The pouch may be sealed to prevent the undesirable release of fragments of the smokeless material into the user's mouth.

According to some embodiments, the pouch may be produced by cutting a sheet of suitable permeable material, which may comprise PLA material, into a desired size.

The cut sheet is folded and the side edges are bonded by a suitable method, such as a heat melt-welding method, high frequency welding method, or ultrasonic welding method, to form the pouch. The top edge may be maintained in an unbonded state, to provide access for inserting the smokeless material into the pouch. After the smokeless material is inserted into the pouch the final seam may be sealed by a suitable method such as one of the above-mentioned welding methods. In preferred embodiments, the sheets are bonded using ultrasonic welding.

A binder may be used to facilitate bonding of the material. The binder may be any suitable adhesive material, and suitable binders will be known to the skilled person. For example, thermoplastic binders based on polyacrylates can be used as suitable polymer binders. Alternatively, cross-linkable systems based on vinyl acetate copolymers can be used.

The binder may comprise a biodegradable material so that the pouch is able to degrade in a natural environment after removal from the mouth of the user and subsequent disposal. If the binder is biodegradable then this may promote disintegration of the smokeless oral product and thus enhanced biodegradation.

Figure 1 shows a method of forming a smokeless oral product comprising a heat-melt welding method. In the embodiment shown, a sheet **1** comprising a mixture of woven and non-woven PO material is folded and the opposite edges **2** and **3** are sealed by heat-melt welding to form a tube, having a longitudinal seam **4**. The bottom **5** of the tube is then sealed by heat-melt welding to form a lateral seam **6**. Smokeless material is then inserted into the tube at the open top end **7**. In a final step, which is sequentially repeated to produce multiple smokeless oral products, the tube is heat-melt welded and cut to yield a smokeless oral product **8** and a tube with a bottom seam **6**'.

In alternative embodiments, the material may be formed in tubular configuration such that a longitudinal seam is not necessary.

Figure 2 shows a pouch formed by a method comprising ultrasonic welding. The method used to form the pouch is analogous to that shown in Figure 1. The pouch **9** is composed of a woven PLA material. As shown in Figure 2, the seams **10** of the pouch are much smaller and more discrete than those of the heat-melt welded pouch shown in Figure 1. Indeed, ultrasonic welding methods may be used to generate seams that are not only smaller, but are more precise, and therefore tidier and more visually appealing. They may also be more comfortable in the mouth of the user. Smaller seams have the further advantage that the amount of woven material required is reduced.

### Pore Size

The pore size of the material comprising the pouch may be selected on the basis of the smokeless material to be used. For example, it is preferable that the pore size of the material is sufficiently small that the amount of any particulate matter that is able to escape the pouch is minimised. On the other hand, the pore size should be large enough to permit free diffusion of water soluble substances across the walls of the pouch.

The chemical nature of the smokeless material may also influence the choice of pore size. For example, if the material in the pouch is relatively hydrophobic, and a very small pore size is used, then the passage of water may be hindered and larger pores may be required.

The ability to regulate the pore size of the material is therefore important. In addition, it may be advantageous to provide a material in which the pores are of a substantially uniform size.

Relative to conventional pouch materials of equivalent mechanical strength, such as fibre web materials, woven materials can have increased porosity. Therefore, the use of woven materials in smokeless oral products can allow enhanced migration of substances from the smokeless material into the mouth. This may be associated with a number of advantages, such as the user being able to obtain a greater concentration of substances from the smokeless material for a particular amount of smokeless material.

Typically the porosity, which is the surface area covered by the pores as a proportion of the total surface area, is greater than 5%, preferably greater than 7%, 10%, 12%, and most preferably is greater than 15%. It is desirable for the porosity of the material to be less than 45%, and is preferably less than 35%, 32%, 30%, and most preferably the porosity is less than 25%.

### Pouch material

The pouch for use in the smokeless oral product is formed from material comprising woven fibres. The fibres comprise a polylactide (PLA) polymer, or a polyolefin (PO) polymer.

The PLA polymer may be prepared by polymerizing lactic acid or lactide.

The PLA polymer may be a homopolymer or a copolymer of the D and L optical isomers. The polymer may be a mixture of homopolymers and/or copolymers. Polyolefin describes any of a class of synthetic resins prepared by the polymerisation of olefins, which are hydrocarbons containing a carbon double-bond, such as (but not limited to) ethylene, propylene, butenes, isoprenes, and pentenes, and copolymers and modifications thereof.

A single polyolefin may be used, or alternatively, the material may comprise a combination of different polyolefins.

The fibres comprising the PLA or PO material may be in the form of multifilaments, monofilaments or staple fibres. The staple fibres may be employed in the form of spun yarns, or in the form of composite yarns comprising the staple fibres and the filaments.

There is no limitation to the cross-sectional profile of the fibres and filaments, however, in general, a circular cross-sectional profile is preferred.

Several techniques can be employed to make the fibres used for production of the pouch material such as melt spinning or dry spinning.

In order to provide the desired flexibility, permeability, and comfort for the user, the thickness of the fibres may be in the range of between 1 and 100 dtex, and optionally between 5 and 50 dtex.

### Woven Material

The fibres are formed into a woven material. The term 'woven' is intended to mean any method of weaving, knitting, or otherwise interlacing fibres or yarns in a regular, repeating arrangement, to form a fabric material.

It may be undesirable for the fibres to be too thin. For example, if the fibres are less than 1 dtex, then slippage of the yarns may occur during production of the woven material. Increasing the yarn density, however reduces the weaving efficiency. In addition, due to the small pore size, the resultant woven material may become easily clogged, resulting in reduced release from the pouch of substances derived from the smokeless material, and this may be undesirable for the user.

Conversely, it may be undesirable for the fibres to be too thick. For example, if the thickness of the fibres is greater than 100 dtex, the resultant woven material may exhibit an increased stiffness and a reduced flexibility, which may result in a pouch that is uncomfortable for the user and causes irritation.

In the woven material, the cover factor K is preferably between 1600 and 6400, and is more preferably between 3200 and 4000. The cover factor K is determined in accordance with the following equation: $K = \left(N \times \left(A\right) < 1 / 2 > / T\right) + \left(M \times \left(B\right) < 1 / 2 > / S\right)$ in which, in respect of woven fabric,
K represents the cover factor of the woven fabric,
N represents the warp density (yarns/10 cm),
M represents the weft density (yarns/10 cm),
A represents the thickness (dtex) of the warp yarns,
B represents the thickness (dtex) of the weft yarns,
T represents the specific gravity of the warp yarns and
S represents the specific gravity of the weft yarns.
   The cover factor K of the woven material correlates with the pore size of the material, wherein the lower the cover value, the greater the pore size. If the cover value for the material is less than 1600, the pore size of the material may be too great. If the cover factor K is greater than 6400, the pore size may be too small and may be prone to clogging.

The thickness of the woven material comprising the pouch is typically greater than 15µm, and may be greater than 20, 35, 50, 80, 100, 120, 150, 175, or 200µm. The pouch material generally has a thickness of less than 500, 450, 400, 350, 300, 250, 200, 150, or 100µm. The woven material may have a thickness in the range of between 50 and 150µm, preferably between 70 and 100µm.

Conventional pouches for smokeless oral tobacco products comprise fibre web material. Due to the orientation of the fibres in such materials, fibre webs have a much greater mechanical strength when stressed in a longitudinal direction versus a lateral (perpendicular) direction. In contrast, woven materials have equal mechanical strength in all directions. This provides greater control and flexibility in the manufacturing process.

In addition, woven materials can have the further advantage of having a surface texture that is pleasant to the touch and may offer the reduced likelihood of irritation in the mouth of the user.

### Non-Woven Materials

In some embodiments, the material comprising the pouch is not a purely woven material, but is a composite material, comprising woven and non-woven material. Such material resembles a combination of woven material and fibre web material.

Generally, the composite material comprises fibres of PO material.

Composite materials comprising woven and non-woven materials may be advantageous as they may be able to be bonded, joined, and/or sealed using methods which are not suitable for use with materials that are exclusively woven or non-woven. For example, composite materials may be sealable by means of ultrasonic or heat treatment, whereas woven PLA material may not be suitable for heat sealing.

In further embodiments, in addition to woven and/or composite materials, the material may also be present in the pouch in the form of a fibre web. The fibre web material may comprise PLA or PO material.

The fibres produced as described above can be converted into non-woven fibre webs by well-known techniques. Alternatively, melt blowing or electro-spinning techniques may also be used and in these methods, a fibre web is produced at the same time the fibre is formed.

### Appearance

Woven PLA and PO materials are generally transparent. Since they have no colour, these materials are resistant to staining. This offers an advantage when used in combination with smokeless material because such material can have a high moisture content. Consequently, materials used in the production of conventional pouches often become stained and discoloured by the action of the moist contents. Such tarnishing of the pouch can be unsightly and unappetising for the user.

The pouch may be coloured. Colour may be imparted to the material by any suitable method. For example, colouring may be added during the manufacture of the fibres comprising the pouch material.

The colour may result in the material having a transparent colouring. Alternatively, the material may have an opaque, entirely coloured, appearance.

Any colour may be used. The colouring may be associated with the particular smokeless tobacco product. For example, if the smokeless oral product contains a mentholated smokeless tobacco material then it may have a green colour.

### Environmental Considerations

PLA is a sustainable alternative to viscose or petrochemical-derived products, since the lactides from which it is ultimately produced can be derived from the fermentation of agricultural by-products such as corn starch or other carbohydrate-rich substances such as maize, sugar, or wheat.

### Additional Materials

The pouch may comprise additional materials in combination with the PLA and/or PO material.

Additional material present in the pouch may comprise woven or non-woven materials, or may comprise a combination of woven and non-woven materials.

The additional material preferably comprises degradable material. For example, polymer groups including polyanhydrides, polyesters (such as those made from diacids and diols), polycarbonates, polyorthoesters, polyphosphazenes, polyesterurethane, polycarbonateurethane, and polyaminoacids, are degradable because they have hydrolysable bonds in the backbone of the polymer chain.

The additional material may comprise a natural polymer such as a polysaccharide, proteins, and polyhydroxybutyrate including its various copolymers.

Another degradable polymer, which may be used as a component of the pouch material, is polyvinylalcohol or its various copolymers.

### Additives

Additives can be applied to the material of the pouch. Such additives could be, for example, where local regulations permit, plasticisers, preservatives, anti-bacterial agents, flavourants, or pharmacological substances.

Additives may be applied in the form of microcapsules, for example, microcapsules comprising liquid flavourants. Alternatively or additionally, additives may be applied in the form of powders, such as powder blended or added to the smokeless material. Additives may also be applied by spray drying. For example, spray-dried flavourant may be applied to the smokeless material prior to incorporation within the pouch.

### Smokeless Material

The 'smokeless material' used herein includes smokeless tobacco material such as Swedish-style snus, and also tobacco substitute materials such as tobacco and nicotine free alternatives to snus.

Nicotine-free alternatives to snus may comprise vegetable fibre portions, flavoured with aromas to imitate the taste of tobacco.

'Tobacco' as used herein includes any part, such as the leaves, flowers, or stems, of any member of the genus Nicotiana and reconstituted materials thereof. It includes derivatives such as specific compounds found in natural tobacco, such as nicotine, whether extracted or synthesized, as well as structural derivatives such as the fibrous portion of a tobacco leaf. It further includes tobacco substitutes which comprise individual chemicals and/or complex chemical entities which, when appropriately prepared, physically resemble natural tobacco.

Tobaccos used in the present invention may include types of tobaccos such as dark air cured tobacco, flue-cured tobacco, burley tobacco, Oriental tobacco, Maryland tobacco, dark tobacco, dark-fired tobacco and Rustica tobaccos, as well as other rare or specialty tobaccos. In preferred embodiments, dark air-cured tobacco is used.

In one embodiment, relatively dry tobacco is ground, sieved and sorted into stem fractions and lamina fractions, each of these being further sorted into small (between about 0.01 to 0.4mm), medium (between about 0.4 to 0.7mm) and large (between about 0.7 to 1.0mm) particles. The desired ratios of particle sizes and tobacco fractions are obtained. The relative amounts of stem to lamina will have some effect on flavour and nicotine delivery, as these components reside most significantly in the lamina portion. Flavour and other characteristics are also influenced by the particular tobacco type used and the curing method it has undergone. For tobacco types which are provided with no distinction between stem and lamina, Rustica or Oriental for example, there may be only a separation of tobacco particles by size.

The relative ratios of particle sizes may affect the final product, making it relatively drier or moister/stickier. The tobacco used may comprise an approximately equal proportion of stem to lamina fractions, or may comprise a larger proportion of lamina than stem. Typical snus products generally contain a full spectrum of particle sizes to effectively release nicotine in a reasonable amount of time, while maintaining structural integrity.

The blend of tobacco particles is mixed with water and, typically, salt. Residual moisture from the tobacco and the added water combine to raise the moisture levels of the mixture to between 25 and 60%. Salt is one form of flavourant; optionally it may be excluded and/or another flavourant may be added at this stage.

The amount of tobacco within the tobacco formulation may vary. The amount of tobacco within the tobacco formulation may be from at least about 25% to at least about 40%, on a dry weight basis.

### Additives to the Smokeless Material

The smokeless material may further include other components. These components may, for example, be included in order to alter the organoleptic properties of the formulation, contributing to the sensory perception by the consumer. The particular components and the amounts in which they are included in the smokeless material of the present invention will vary depending upon the desired flavour, texture, and other characteristics.

For example, the following components may be included:
(a) flavouring agents;
(b) humectants;
(c) pH adjusters or buffering agents;
(d) disintegration aids;
(e) preservatives; and
(f) colorants.

As used herein, the terms "flavour" and "flavourant" refer to materials which, where local regulations permit, may be used to create a desired taste or aroma in a product. They may include extracts and/or may be imitation, synthetic or natural ingredients or blends thereof. They may be in any suitable form, for example, oil, liquid, or powder.

The smokeless material may comprise sensates in addition to flavourants, and these may include cooling agents and heating agents.

The smokeless material may also comprise at least one humectant, such as glycerol or propylene glycol.

The smokeless material may also comprise at least one pH adjuster or buffering agent, which may include metal hydroxides, such as sodium hydroxide and potassium hydroxide, and other alkali metal buffers such as potassium carbonate, sodium carbonate and sodium bicarbonate.

The smokeless material may also comprise at least one preservative, such as potassium sorbate.

## Claims

1. A smokeless oral product (8; 9), comprising:
a single permeable pouch comprising a woven material, and
smokeless material contained in the pouch,
wherein the permeable pouch comprises fibres comprising polylactide material or polyolefin material.

2. A smokeless oral product according to claim 1, wherein the permeable pouch comprises a composite material comprising both woven and non-woven material.

3. A smokeless oral product according to claim 1 or claim 2, wherein the smokeless material comprises smokeless tobacco material.

4. A smokeless oral product according to claim 3, wherein the smokeless tobacco material is Swedish-style snus.

5. A smokeless oral product according claim 1 or 2, wherein the smokeless material comprises tobacco substitute material which is tobacco and nicotine free.

6. A method of producing a smokeless oral product (8; 9), comprising providing a single permeable pouch comprising a woven polymer material, wherein the permeable pouch comprises fibres comprising polylactide material or polyolefin material and wherein the permeable pouch comprises smokeless material contained in the pouch.

7. A method according to claim 6, comprising sealing the material using a heat-melt welding technique.

8. A method according to claim 6, comprising sealing the material using an ultrasonic welding technique.

## Patentansprüche

1. Rauchloses Oralprodukt (8; 9), umfassend:
einen einzelnen durchlässigen Beutel, der ein gewebtes Material umfasst, und
rauchloses Material, das in dem Beutel enthalten ist,
wobei der durchlässige Beutel Fasern umfasst, die Polylactidmaterial oder Polyolefinmaterial umfassen.

2. Rauchloses Oralprodukt gemäß Anspruch 1, wobei der durchlässige Beutel ein Verbundmaterial umfasst, das sowohl gewebtes als auch nichtgewebtes Material umfasst.

3. Rauchloses Oralprodukt gemäß Anspruch 1 oder Anspruch 2, wobei das rauchlose Material rauchloses Tabakmaterial umfasst.

4. Rauchloses Oralprodukt gemäß Anspruch 3, wobei das rauchlose Tabakmaterial Snus von schwedischer Art ist.

5. Rauchloses Oralprodukt gemäß Anspruch 1 oder 2, wobei das rauchlose Material Tabakersatzmaterial umfasst, das tabak- und nikotinfrei ist.

6. Verfahren zur Herstellung eines rauchlosen Oralprodukts (8; 9), umfassend Bereitstellen eines einzelnen durchlässigen Beutels, der ein gewebtes Polymermaterial umfasst, wobei der durchlässige Beutel Fasern umfasst, die Polylactidmaterial oder Polyolefinmaterial umfassen, und wobei der durchlässige Beutel rauchloses Material umfasst, das in dem Beutel enthalten ist.

7. Verfahren gemäß Anspruch 6, umfassend Siegeln des Materials unter Verwendung eines Heißschmelz-Schweißverfahrens.

8. Verfahren gemäß Anspruch 6, umfassend Siegeln des Materials unter Verwendung eines Ultraschall-Schweißverfahrens.

## Revendications

1. Produit oral sans fumée (8 ; 9), comprenant :
une poche perméable unique comprenant un matériau tissé, et
un matériau sans fumée contenu dans la poche,
dans lequel la poche perméable comprend des fibres comprenant un matériau polylactide ou un matériau polyoléfine.

2. Produit oral sans fumée selon la revendication 1, dans lequel la poche perméable comprend un matériau composite comprenant à la fois un matériau tissé et un matériau non tissé.

3. Produit oral sans fumée selon la revendication 1 ou la revendication 2, dans lequel le matériau sans fumée comprend un matériau de type tabac sans fumée.

4. Produit oral sans fumée selon la revendication 3, dans lequel le matériau de type tabac sans fumée est un snus de style suédois.

5. Produit oral sans fumée selon la revendication 1 ou 2, dans lequel le matériau sans fumée comprend un matériau de substitution du tabac qui ne contient pas de tabac ni de nicotine.

6. Procédé de fabrication d'un produit oral sans fumée (8; 9), comprenant la fourniture d'une poche perméable unique comprenant un matériau polymère tissé, dans lequel la poche perméable comprend des fibres comprenant un matériau polylactide ou un matériau polyoléfine et dans lequel la poche perméable comprend un matériau sans fumée contenu dans la poche.

7. Procédé selon la revendication 6, comprenant le fait d'enfermer hermétiquement le matériau en utilisant une technique de soudage par fusion thermique.

8. Procédé selon la revendication 6, comprenant le fait d'enfermer hermétiquement le matériau en utilisant une technique de soudage ultrasonique.
